

## UNITED STATES PATENT OFFICE

2,665,207

## NAPHTHENATE SIZED PRODUCTS

Frank M. McMillan, Berkeley, and Robert D. Sullivan, Oakland, Calif., assignors to Shell Development Company, San Francisco, Calif., a corporation of Delaware

No Drawing. Application June 29, 1948,  
Serial No. 35,988

6 Claims. (Cl. 92—3)

1

This invention relates to an improved method of sizing fibrous materials such as paper, cardboard, textile threads, fabrics and the like. It deals with a new process whereby such materials may be sized more efficiently and economically and with the sized products of more advantageous properties thereby obtained.

Rosin, paraffin wax, natural and synthetic resins, asphalt, tars and a great many other materials have been suggested as suitable materials for sizing paper or the like. All of these sizing materials have disadvantages of one kind or another, some being more expensive than is desirable and others being of inadequate waterproofing ability or having other characteristics which limit their usefulness. It is an important object of the present invention to provide a method of sizing which overcomes these disadvantages of prior sizes and which will be more economical in commercial practice. Another object is to provide improved articles of manufacture particularly sized paper and the like, which are more water-resistant than prior products of a similar type. Still other objects and advantages of the invention will be apparent from the following description of the invention in some of its more preferred forms, it being understood that the invention is not limited thereto but is broadly applicable and capable of many variations.

It has been found that fibrous materials, particularly fibers of cellulose and the like, may be advantageously sized with salts of naphthenic acids of low molecular weight having high acid numbers, i. e., acid numbers of 200 or greater, preferably acid numbers of about 225 to 400. The ordinary naphthenates of commerce are thus not suitable for use according to the invention since they generally contain undesirably large amounts of naphthenic acids having acid numbers of less than 200. However, naphthenates of the required characteristics may be obtained from commercial naphthenate mixtures by treatment with acid to form the free naphthenic acids followed by distillation of the latter to take off a fraction having the desired high acid number. Especially advantageous sources of naphthenates having desirable sizing properties are those obtainable in the refining of properly selected fractions of petroleum such, for example, as gasoline or kerosene fractions, gas oil or the like. Methods which may be used in obtaining the naphthenates from such sources include, for example, alkali treatment of acid-refined petroleum distillates, or the caustic distillation of mineral oils, particularly oils from Texas and California crudes, to obtain

oil-containing naphthenates which may be used as such or may be partially purified by acid treatment or more completely deoiled by dispersion in an aqueous medium followed by de-emulsification in the presence of a solvent for the oil. Where more highly purified naphthenates are desired, they may be produced by known methods, including washing with sea water or treatment to remove sulfur compounds, for example. It is not necessary, however, that the naphthenates of naphthenic acids having acid numbers greater than 200 be used in pure form since it is quite feasible to use them with hydrocarbons including the hydrocarbons from which they are derived. Indeed, it is quite feasible to employ the naphthenates according to the invention along with other materials which may or may not have sizing properties of their own. Most preferably, other sizing materials such, for example, as rosin size or higher boiling hydrocarbons are used when the naphthenates of naphthenic acids of high acid number are employed in the form of mixtures with other materials.

The naphthenates are preferably used as the sodium salts since they are generally less expensive and have desirable solubility characteristics. However, other alkali metal salts, particularly the potassium salts, may also be employed as may also alkaline earth metal salts, such as the calcium and magnesium salts, aluminum salts or other inorganic salts. When using aluminum and like water-insoluble salts it is desirable to use an emulsifying agent for the naphthenate salt to insure its uniform distribution on the fibers. To this end, a small amount, usually about 0.1% to 5% by weight of the total amount of sizing agent employed, of a suitable soap is preferably used. Fatty acid soaps, higher alkyl sulfate salts, organic sulfonic acid salts particularly alkyl aryl sulfonates, naphthenates of naphthenic acids having acid numbers less than 200, sodium rosinate, and the like are suitable. For certain purposes it may be desirable to use ammonium or amine salts of the naphthenic acids of acid number 200 or greater. Water-soluble amines such, for instance, as dimethylamine, propylamine, cyclohexylamine, the ethanolamines, etc. are suitable for forming naphthenates which may be used in the process of the invention.

The naphthenates corresponding to naphthenic acids of acid number 200 to 400 or more may be used simply and efficiently for sizing fibers, for example, by adding the naphthenate to an aqueous slurry of the fibers and, after stirring to insure uniform distribution of the naphthenate

size and fibers, precipitating the sizing agent with a suitable precipitant such as paper maker's alum or the like. The naphthenates of high acid number naphthenic acids thus have the advantage not only of imparting exceptional water resistance to cellulose fibers and the like, but also of being adapted to ready use in the same equipment as conventional sizes. Thus, in sizing paper according to the invention, for instance, a sodium naphthenate of a naphthenic acid of acid number 200 to 400 may be added to any suitable paper pulp in the beater engine at any stage of beating, although as a rule it is more advantageously introduced when the beating has been substantially completed, or the sizing may be carried out in the Jordan machines or at the screens. A wide range of precipitants may be used for fixing the naphthenate sizes on the fibers. Alum, aluminum sulfate, aluminum chloride, calcium chloride, acids such as sulfuric or hydrochloric acid, and the like are suitable. The precipitant may be added to the fiber before or along with the naphthenate size but generally it is preferred to add it a sufficient time after adding the size to provide an adequate interval for uniform distribution of the size before introduction of the precipitant. A pH of about 4.5 to 6, depending on the type of pulp, is desirable during precipitation. If necessary, the pH may be controlled by adding dilute acid in the beater. About 25 grams of aluminum sulfate per kilogram of dry stuff in the beater gives satisfactory precipitation. Too much aluminum in the paper should be avoided as it adversely affects the permeability to water and the age resistance of the paper.

The amount of naphthenate size which it will be most advantageous to employ will depend on the nature of the fibrous material being treated, the purpose for which it is intended, the type of naphthenate chosen, and the method of its application. As little as 0.2% based on the dry weight of the paper is effective, but up to 10% or more may be used, the preferred range being usually about 0.5% to about 3%.

As previously pointed out, it may sometimes be desirable to use the naphthenates of high acid number naphthenic acids in conjunction with other sizing materials. Thus, emulsions of oils or waxes such as paraffin, ceresin and montan waxes, for example, are useful when used in combination with high acid number naphthenates. Hydrocarbons such as lubricating oils, spindle oil, asphalts, bitumens, etc. may likewise be used. However, there are special advantages in using cyclic extracts of predominantly aromatic and naphthenic nature, such as are obtainable by extracting petroleum or related oils, including hydrogenation products of coal and the like, with solvents which are selective for non-paraffinic constituents. A wide variety of polar solvents may be used for the preparation of such extracts, liquid sulfur dioxide, phenol, cresylic acid, furfural, beta,beta-dichlorethyl ether, nitrobenzene, the sulfolanes and sulfolenes, and the like being typical examples of suitable solvents which may be advantageously used. Combinations of solvents, as phenol with cresylic acid or liquid sulfur dioxide with benzene or toluene, for instance, are useful and the use of the so-called double solvent process employing mutually immiscible solvents, e. g. cresylic acid with propane, also gives suitable extracts. Extracts of heavier petroleum oils such as the lubricating oils and residual stocks are especially useful in conjunction with high acid number naphthenates in ac-

cordance with the invention, but other fractions of petroleum or related hydrocarbon products can also be used successfully as sources of the extracts. The extracts may be derived, for example, from lubricant distillates or bright oils or cylinder stocks which may, for instance, range in gravity from 15° to 8° API at 60° F. They may be obtained from any mixed type petroleum oil such as Mid-Continent or Coastal or California crude or, in lower yields, from Pennsylvania type oils. For use in sizing in combination with naphthenates of high acid number naphthenic acids, extracts boiling above 300° C. at 760 mm. Hg. pressure are preferred, and most preferably extracts boiling from about 125° C. to 300° C. at 1 mm. Hg. pressure are used. The more viscous extracts usually give emulsions with the most desirable sizing properties. For this reason extracts within the viscosity range of about 75 to 5000 at 210° F., S. U. S., have advantages. It is often advantageous to fractionate the initial extract to separate fractions of especially advantageous properties; thus, for instance, it has been found that the higher boiling 50% to 75% of an Edeleanu extract of lubricating oil gives superior sizing when used with naphthenates according to the invention.

The proportion of naphthenate of high acid number to hydrocarbon used when employing such mixtures for paper sizing according to the invention can be varied but as a rule will be such as corresponds to about 25% to about 99%, more preferably 50% to 99%, by weight of naphthenate based on the total weight of naphthenate and hydrocarbon. Such hydrocarbon should be used in the form of an aqueous emulsion; to which end a small amount, usually about 2% to 10% by weight of the naphthenate and hydrocarbon present, of an emulsifying agent should be employed. Soap, alkyl sulfate salts, sulfonic acid salts, particularly alkyl aryl sulfonates, sodium rosinate and the like may be used as emulsifying agents. The most advantageous sizing emulsions, however, are those made from naphthenates without other emulsifying agents.

The following example shows the results obtainable according to the invention in comparison with sizing with naphthenates of low acid number naphthenic acids.

#### Example

Deoiled naphthenates were used as the sole sizing agent for kraft pulp. The deoiled naphthenic acids were completely saponified with sodium hydroxide solution to form a 10% aqueous solution of sodium naphthenate. The oil content of the deoiled naphthenates was between 3% and 10% by weight. About 2% of sodium naphthenate based upon the dry weight of pulp was used and the beaten pulp was stirred for 15 minutes with the naphthenates before adding 3% of paper maker's alum as precipitant, after which 15 minutes additional stirring was given the pulp. Comparative tests were carried out on sheets made from the two pulps thus sized. The sheets were prepared in a standard hand mold, followed by pressing at 50 pounds for 2 minutes. The sheets were dried at 60° C.-70° C. and tested after conditioning the test samples at 70° F. and 50% relative humidity. The resulting sheets were compared as to wetting time (i. e., time for the paper floating on water to show wet spots on its upper surface) and ink absorption (i. e., the area stained by 0.05 ml. of ink dropped on the surface and allowed to dry). As shown by the following

results, the naphthenates of higher acid number were by far the superior sizing agents.

| Acid No. of Naphthenate | Water Wetting Time of Paper (hours) | Absorption of Ink (area of dry spot, mm. <sup>2</sup> ) |
|-------------------------|-------------------------------------|---------------------------------------------------------|
| blank                   | <0.05                               | 190                                                     |
| 150                     | 0.5                                 | 112                                                     |
| 200                     | 48.                                 | 72                                                      |

Similar good results are obtained when sulfite pulp is substituted for the kraft pulp.

It will thus be seen that the new process of the invention offers many advantages over prior methods of sizing and gives sized products of superior properties. It will also be apparent that the invention is not limited to the applications given by way of illustration nor to details of operation disclosed. Thus, for example, instead of the naphthenic acid salts, the corresponding free naphthenic acids having acid numbers of 200 or greater, preferably 225 to 400, may be used as the sizing agent and these naphthenic acids and their salts will be referred to generically hereinafter as naphthenates. Still other variations may be made in the process of the invention which will be understood as not dependent upon any theory advanced in explanation of the improved results which are obtained.

We claim as our invention:

1. A paper product comprising sized cellulose fibers containing about 0.5% to about 5% by weight of sizing agent wherein the effective sizing agent is essentially naphthenates of naphthenic acids having an average acid number greater than 200 but not greater than about 400, together with a mixture of cyclic components of petroleum soluble in solvents which are selective for non-paraffinic constituents thereof.
2. A paper product comprising cellulose fibers having distributed on their surface about 1% to about 5% by weight of the dry fibers of a naphthenate of a naphthenic acid having an acid number of 225 to 400, together with cyclic constituents of a lubricating oil fraction of petroleum soluble in solvents which are selective for non-paraffinic constituents in proportions such that the naphthenates correspond to about 25% to 97% of the total weight of naphthenates and said cyclic constituents.

3. A fibrous product comprising sized cellulose fibers having distributed on their surface 0.2% to about 10% by weight of the dried fibers of naphthenates of naphthenic acids having an average acid number greater than 200 but not greater than about 400, together with a mixture of cyclic components of petroleum soluble in solvents which are selective for non-paraffinic constituents thereof.
- 10 4. A fibrous product in accordance with claim 3 wherein the sized fibers are kraft paper pulp fibers, and said cyclic components are derived from a lubricating oil fraction of petroleum.
- 15 5. A fibrous product in accordance with claim 3 wherein the naphthenates are sodium naphthenates essentially derived from naphthenic acids having acid numbers of at least 225 but not greater than 400.
- 20 6. A fibrous product in accordance with claim 3 wherein said cyclic components are derived from a lubricating oil fraction of petroleum and are present in proportions such that the naphthenates correspond to about 25% to 99% of the total weight of naphthenates and said cyclic components.

FRANK M. McMILLAN.  
ROBERT D. SULLIVAN.

References Cited in the file of this patent

UNITED STATES PATENTS

| Number       | Name                 | Date          |
|--------------|----------------------|---------------|
| 1,519,803    | Sellers et al. ----- | Dec. 16, 1924 |
| 1,920,483    | Senftner -----       | Aug. 1, 1933  |
| 2,332,226    | Hutchins -----       | Oct. 19, 1943 |
| 35 2,340,035 | Zimmer et al. -----  | Jan. 25, 1944 |
| 2,377,359    | Musher -----         | June 5, 1945  |
| 2,423,619    | Roon -----           | July 8, 1947  |
| 2,447,475    | Kaberg et al. -----  | Aug. 17, 1948 |
| 40 2,538,742 | Willey -----         | Jan. 16, 1951 |

FOREIGN PATENTS

| Number  | Country             | Date          |
|---------|---------------------|---------------|
| 364,564 | Germany -----       | Nov. 27, 1922 |
| 525,338 | Great Britain ----- | Aug. 27, 1940 |

OTHER REFERENCES

- Gershzon, Chemical Abstract, vol. 33, p. 8989.  
Gershzon, Chemical Abstract, vol. 34, p. 3119.  
Chemical Reviews, vol. 30, pages 97-111 (1942).